

## UNITED STATES PATENT OFFICE

2,675,360

CELLULOSE ACETATE FIBERS WITH  
IMPROVED DYEING PROPERTIESJohn R. Caldwell, Kingsport, Tenn., assignor to  
Eastman Kodak Company, Rochester, N. Y., a  
corporation of New JerseyNo Drawing. Application April 1, 1952,  
Serial No. 279,963

11 Claims. (Cl. 260—13)

1

This invention relates to the manufacture of synthetic fibers from the lower fatty esters of cellulose, and more particularly to the manufacture of cellulose acetate fibers having an improved affinity for acid wool dyes.

In the textile industry it is often desirable to use fibers of different kinds in the manufacture of fabrics. After the fabric has been woven, it may then be subjected to a dyeing operation and it is often desirable that the fibers have dyeing properties which are substantially equivalent. In those fabrics in which cellulose ester fibers are combined with the fibers of natural wool, it has commonly been necessary heretofore to employ both an acetate dyestuff and a wool dyestuff to impart color to the fabric. In many cases considerable difficulty has been encountered in matching the shades of the wool fibers and the cellulose ester fibers. In addition, the two types of dyestuffs often respond differently to laundering, light fading, etc. resulting in fabrics having a spotty or irregular appearance after they have been exposed to conditions of wear and cleaning.

Many attempts have been made heretofore to impart properties to cellulose ester fibers so they are receptive to acid type dyes, but the results obtained have not been too satisfactory. It is thought that the dyeing of wool fibers by acid-type dyestuffs takes place through the reaction of the sulfonic acid groups in the dye molecule with amine groups in the wool to form a salt linkage. To impart wool dye affinity to cellulose ester fibers, compounds have been incorporated therein having basic amino groups, resembling those present in natural wool. In most cases heretofore the fibers which have been so prepared would take up only small amounts of dyestuffs to give a weak shade, or the dye employed to dye the cellulose ester fibers would show poor stability toward light fading and laundering.

An object of my invention is to prepare fibers of the lower fatty esters of cellulose having good susceptibility to acid dyes and good stability, when so dyed, to fading by light or by laundering.

Another object of the invention is to provide cellulose acetate fibers than can be dyed readily with acid wool dyes.

Still another object of the invention is to provide compositions containing cellulose acetate and linear polymeric urethanes in an intimate mixture.

Other objects of my invention are apparent hereinafter.

In accordance with the invention these and

2

other objects are attained by incorporating linear polyurethanes in cellulose ester spinning dopes and converting the solution to fibers. The presence of the linear polyurethanes in the fiber imparts acid wool dyeing properties thereto. Fibers prepared in this way can be colored deep shades by acid wool dyes applied by standard methods. It is not necessary to use swelling agents or solvents in the dye bath.

10 The linear polyurethanes employed in accordance with my invention contain tertiary amine groups which cause the cellulose ester fibers containing them to have a strong affinity for acid wool dyes. The polyurethanes may be made by reacting triamines containing one tertiary amino group with dichlorocarbonates of glycols. The reaction may be represented by the general equation:



wherein R is an alkyl group containing 1 to 4 carbon atoms, e. g. methyl, ethyl, propyl, isopropyl, and butyl; X is a straight or branched alkylene chain containing 2 to 6 carbon atoms e. g.



n is 2, 3 or 4, and m is a whole number from 20 to 200.

35 The amines used in the process are prepared by known methods. For example, a particularly useful amine is obtained by adding two mols of acrylonitrile to one mol of methyl amine and hydrogenating the two nitrile groups to primary amine groups. The product is methyl bis (gamma-aminopropyl) amine and has the structure



40 45 The dichlorocarbonates are made by treating glycols with excess phosgene at about  $-10^\circ\text{C}$ .

The reaction between the dichlorocarbonate and amino compound is carried out in an inert liquid such as benzene, toluene, ethylene dichloride or dioxane. An alkali such as sodium hydroxide, sodium carbonate or calcium oxide is used to combine with the liberated HCl.

50 55 The most desirable means of preparing cellulose ester fibers in accordance with my invention is by dissolving the linear polyurethane in the



2 to 4, and  $m$  is a whole number from 20 to 200. 2. A spinning solution essentially consisting of a lower fatty acid of cellulose having 1 to 4 carbon atoms and approximately 10 to 40% by weight of a linear polyurethane having the general formula:



wherein R is a member selected from the class consisting of methyl, ethyl, propyl, isopropyl and butyl, X is an alkylene group selected from the class consisting of alkylene groups having 2 to 6 carbon atoms,  $n$  is a small whole number from 2 to 4, and  $m$  is a whole number from 20 to 200, dissolved in a low boiling volatile organic solvent.

3. Cellulose ester fibers having wool dyeing properties essentially consisting of a lower fatty acid ester of cellulose having 1 to 4 carbon atoms and approximately 10 to 40% of the linear polyurethane having the formula:



wherein  $m$  is a whole number from 20 to 200.

4. Cellulose ester fibers having wool dyeing properties essentially consisting of a lower fatty acid ester of cellulose having 1 to 4 carbon atoms and approximately 10 to 40% of the linear polyurethane having the formula:



wherein  $m$  is a whole number from 20 to 200.

5. Cellulose ester fibers having wool dyeing properties essentially consisting of a lower fatty acid ester of cellulose having 1 to 4 carbon atoms and approximately 10 to 40% of the linear polyurethane having the formula:



wherein  $m$  is a whole number from 20 to 200.

6. A spinning solution essentially consisting of cellulose acetate and approximately 10 to 40% of the linear polyurethane having the formula:



wherein  $m$  is a whole number from 20 to 200 dissolved in acetone.

7. A spinning solution essentially consisting of cellulose acetate and approximately 10 to 40% of the linear polyurethane having the formula:



wherein  $m$  is a whole number from 20 to 200 dissolved in acetone.

8. A spinning solution essentially consisting of cellulose acetate and approximately 10 to 40% of the linear polyurethane having the formula:



15 wherein  $m$  is a whole number from 20 to 200 dissolved in acetone.

9. Fibers having wool dyeing properties essentially consisting of cellulose acetate and approximately 10 to 40% of the linear polyurethane having the formula:



wherein  $m$  is a whole number from 20 to 200.

10. Fibers having wool dyeing properties essentially consisting of cellulose acetate and approximately 10 to 40% of the linear polyurethane having the formula:



wherein  $m$  is a whole number from 20 to 200.

11. Fibers having wool dyeing properties essentially consisting of cellulose acetate and approximately 10 to 40% of the linear polyurethane having the formula:



40 wherein  $m$  is a whole number from 20 to 200.

#### References Cited in the file of this patent

#### UNITED STATES PATENTS

|           |               |               |
|-----------|---------------|---------------|
| Number    | Name          | Date          |
| 2,356,079 | Nelles et al. | Aug. 15, 1944 |

#### FOREIGN PATENTS

|               |               |
|---------------|---------------|
| Country       | Date          |
| Great Britain | Jan. 13, 1949 |